

## [54] PROCESS FOR PRODUCING CRIMPED POLYESTER FILAMENTS

[75] Inventors: Nobuharu Izawa; Munetsugu Kikuyama; Hiroshi Toyoshima; Ryuji Yamamoto, Yasuhiro Murase; all of Matsuyama, Japan

[73] Assignee: Teijin Limited, Osaka, Japan

[22] Filed: May 4, 1971

[21] Appl. No.: 140,209

[52] U.S. Cl.....28/72.14

[51] Int. Cl. ....D02g 1/12

[58] Field of Search.....28/1.6, 72.14

## [56] References Cited

## UNITED STATES PATENTS

3,553,803 1/1971 Buschmann et al. ....28/1.6

Primary Examiner—Louis K. Rimrodt  
Attorney—Sherman & Shalloway

## [57] ABSTRACT

A process for producing polyester filaments having high Young's modulus and excellent crimps, which comprises heat-treating a bundle of drawn filaments of linear polyester in which at least 85 mole percent of the recurring units consist of ethylene terephthalate, at a temperature of 135° to 240°C. under a tension of at least 0.3 g/denier, feeding the filaments to the nip rollers of a stuffer box while maintaining the filaments at a temperature at least 10°C. lower than the heat-treating temperature and between 100° and 140°C. under a tension of at least 0.1 g/denier, crimping the filaments in the stuffer box, and then with-drawing the filaments from the stuffer box.

8 Claims, 1 Drawing Figure



PATENTED MAR 13 1973

3,719,976



## PROCESS FOR PRODUCING CRIMPED POLYESTER FILAMENTS

This invention relates to a process for producing polyester filaments having both high Young's modulus and excellent crimps.

Previously, polyester type fibers have been widely utilized in the form of staple fibers after being given mechanical crimps. Usually, after melt spinning, the polyester fibers obtained are drawn, and then subjected to heat-treatment while allowing shrinkage to take place in order to improve their dimensional stability, but the Young's modulus of the polyester fibers thus obtained is considerably lower than that of natural cotton fibers. Therefore, there has been a demand for excellently crimped polyester fibers still having a Young's modulus equal to, or higher than, natural cotton fibers. In an attempt to produce such polyester fibers, a method has been developed in which after melt spinning, the resulting filaments are drawn in multi-stages at the highest possible draw ratios to form polyester filaments having a high Young's modulus, and then the filaments are subjected to a crimping treatment. However, when such filaments are crimped, for instance, by a stuffer crimper, there is the defect that the filaments are more difficult to crimp with increasing Young's modulus. This is due to the fact that the deformation of the filaments is difficult to cause because of the high Young's modulus, and the filaments are not sufficiently bent. One method of removing this defect is proposed in Japanese Patent Publication No. 22028/64 which discloses a method wherein the filaments are preheated before the crimping operation so as to reduce the Young's modulus and accordingly to make them easy to crimp. Another method of this kind is disclosed in Japanese Patent Publication No. 14017/64, in which after heat-treatment under tension, the filaments are cooled to below the minimum crystallization temperature (usually 90°-95°C. for polyester fibers) to retard crystallization. These methods have contributed to some extent to the improvement of the crimpability of the polyester fibers of high Young's modulus. But the crimpability is still inferior to that of polyester filaments having low Young's modulus, and improvement is still required.

It is therefore an object of this invention to provide a process for producing polyester filaments having high Young's modulus and excellent crimps which properties have been somewhat inconsistent with each other.

According to this invention, a process is provided for producing polyester filaments having high Young's modulus and excellent crimps, which comprises heat-treating a bundle of drawn filaments of a substantially linear, fiber-forming, high-molecular-weight polyester having at least 85 mole percent of the recurring units consisting of ethylene terephthalate, at a temperature of 135° to 240°C. under a tension of at least 0.3 g/denier, feeding the filaments to nip rollers of a stuffer crimper while maintaining the filaments at a temperature at least 10°C. lower than the heat-treating temperature and between 100° and 140°C. under a tension of 0.1 g/denier or more, crimping the filaments in the stuffer box and then withdrawing the filaments therefrom.

The invention will be described in greater detail below with reference to the accompanying drawing

which is a schematic side elevation of an apparatus for performing one embodiment of the process of the present invention.

The polyester filaments used in the invention are those obtained from a substantially linear, fiber-forming, high-molecular-weight polyester in which at least 85 mole percent of the recurring units consist of ethylene terephthalate. The polyester polymer may contain less than 15 mole percent of an acid component such as isophthalic acid or adipic acid, an alcohol component such as propylene glycol, or a branching agent as a copolymerizable component.

According to the process of the present invention, the polyester described above is melt-spun by an ordinary method to form undrawn filaments and then the undrawn filaments are hot drawn by a known method to form drawn filaments. Preferably, the drawing is carried out in multi-stages, and by this method highly oriented filaments can be obtained. The preferred total draw ratio used at this time is 3.5 to 6.0. The drawn filaments so obtained are heat treated at a temperature of 135° to 240°C. under a tension of at least 0.3 g/denier to produce polyester filaments having high Young's modulus which are highly oriented and crystallized. If the heat-treatment temperature is lower than 135°C., the Young's modulus of the resulting crimped filaments is not sufficiently high. On the other hand, heat-treating temperatures above 240°C. cause localized melting of the filaments, and result in the melt-adhesion of the filaments with one another. Such filaments are of course not viable for practical purposes.

The preferred heat-treating temperature is from 150° to 230°C. The tension to be exerted on the filaments at the time of heat-treatment should be at least 0.3 g/denier. If the tension is lower than 0.3 g/denier, even heat-treatment at temperatures within the above-specified range does not give filaments of sufficiently high Young's modulus, and there is the accompanying defect of the difficulty of crimping such filaments. The preferred lower limit of the tension is 0.5 g/denier, and the preferred upper limit is 3.5 g/denier.

The heat-treated polyester filaments are then cooled, and then fed to nip rollers of a stuffer box while the filaments immediately before entry into the nip rollers are maintained at a temperature at least 10°C. preferably at least 20°C. lower than the heat-treatment temperature and between 100° and 140°C. and under a tension of at least 0.1 g/denier. Within the stuffer box, the filaments are crimped in a manner known per se. The crimped filaments are withdrawn from the stuffer box in accordance with a customary method. Conveniently, the temperature adjustment of the filaments is accomplished by using conventional heating rollers. The temperature of the filaments generally drops to some extent during the travelling of the filaments between the last heating roller and the nip rollers of the stuffer crimper. In the process of the present invention, therefore, it is necessary to set the temperature of the heating rollers so that the temperature of the filaments immediately before entry into the nip rollers is within the range specified above. The extent of temperature drop of the filaments travelling between the last heating roller and the nip rollers depends upon such factors as the difference between the temperature of the last heating roller and the ambient temperature or the

travelling time (usually less than several seconds), but once the operational conditions are set at constant values, the extent of the temperature drop also becomes substantially constant. Therefore, in actual operation, the temperature of the filaments immediately before entry into the nip rollers is measured by a proper surface temperature measuring device, and the temperature of the heating roller is set so that this measured temperature is within the temperature specified in the present invention.

The critical point of the process of the invention is that the polyester filaments heat-treated under tension are cooled to a temperature at least 10°C. lower than the heat-treating temperature and between 100° and 140°C. and placed under a tension of at least 0.1 g/denier, and in this state the filaments are fed to the nip rollers of the stuffer crisper. In particular, the novel feature of the invention consists in the employment of the above-described feed conditions in relation to the condition of heat treatment under tension mentioned above.

When the polyester filaments are stuffed into the stuffer box via the nip rollers, they are inevitably released from tension within the stuffer box. As is generally known, when filaments are placed under tension, free shrinkage is restrained by the tension, but when the filaments are placed in a tension free state, free shrinkage develops abruptly and easily; consequently, the orientation of the filaments is relaxed and their Young's modulus is reduced. Such a relaxation of the orientation which occurs within the stuffer box is supposed to be higher with increasing temperature of the filaments fed into the stuffer box. It has been found that in order to prevent the high Young's modulus of the polyester filaments attained by the heat-treatment specified in the present invention, from being reduced by the relaxation of the orientation described above, it is very effective to feed the filaments to the nip rollers of a stuffer box while maintaining the filaments at a temperature at least 10°C., preferably at least 20°C., lower than the heat-treatment temperature.

For the same reason as mentioned above, too high a temperature of the filaments at the entry into the stuffer box is undesirable for maintaining a high Young's modulus. It is therefore necessary to adjust the temperature of the filaments to be fed to the nip rollers by the process of the invention to 140°C. or below. On the other hand, from the standpoint of the ease of crimping, filaments to be crimped should conveniently have the highest possible temperature and be softened. Since the filaments to be crimped in the invention have high Young's modulus and are highly oriented and crystallized, the softening of the filaments plays an especially important role for imparting good crimps to the filaments. Therefore, in the process of the invention, the temperature of the filaments to be fed to the nip rollers should be adjusted to 100°C. or above, preferably 110°C. or above.

It is further very important in the process of the present invention that the polyester filaments heat-treated under tension should be fed to the nip rollers of the stuffer box while maintaining them under a tension of at least 0.1 g/denier without releasing the tension. In the conventional methods, it was common practice to release the tension of filaments and place them in a ten-

sion-free state or place them under a slight tension, and feed the filament into the stuffer box in such a tension-free state. According to these methods, the fiber-structure of the filaments is stabilized incident to their shrinkage in a state of low tension. On the other hand, the degree of orientation is reduced, and the Young's modulus of the filaments is decreased. It is due to this structural stabilization by the shrinkage that the filaments become difficult to crimp. The novel feature of the process of the present invention is that the filaments can be given both excellent crimps and a high level of Young's modulus by placing the heat-treated filaments under tension until they are fed into the stuffer box and at the same time maintaining the filaments immediately before entry into the nip rollers at the specific temperature described above. In the process of the present invention, the preferred tension to be exerted on the filaments to be fed to the nip rollers is at least 0.2 g/denier. The upper limit of the tension is difficult to set, but can be defined as the tension such that the nip rollers of the stuffer box can grip the filaments sufficiently without slippage. Usually, the upper limit of the tension is about 1.0 g/denier. The stuffer crisper used in the invention may be of any type known and used in the art.

Referring to the accompanying drawing, undrawn filaments extruded from a melt-spinning apparatus of the conventional type (not shown) are drawn by feed rollers (not shown), a heating device (not shown) such as hot pin, hot plate, or hot bath and a pair of draw rollers 1 and 1' to produce drawn filaments 2. The drawn filaments 2 which have left a pair of draw rollers 1 and 1', are heat-treated under tension by rollers 3, 4, 5, 6 and 7 heated at 135°-240°C. The filaments are then passed over heating rollers 8 and 9 the temperature of which is set so that the temperature of the filaments immediately before entry into between nip rollers 11 and 11' is at least 10°C. lower than the heat-treating temperature and between 100° and 140°C., and cooled to some extent. The filaments are then passed over a guide roller 10, and then fed between a pair of nip rollers 11 and 11' and then stuffed into a stuffer box 12 and crimped therein. Thereafter, the crimped filaments are withdrawn from the stuffer box 12, and fed onto a net conveyor 13. If desired, the filaments are subjected to heat-treatment in a relaxed state. Then the filaments are transferred to a cutter (not shown), and cut to staple fibers. It is preferred that the draw rollers 1 and 1' and the heating rollers 3 to 9 are all driven at the same peripheral speed. The peripheral speed of the nip rollers 11 and 11' may be 95-105 percent of that of the heating roller 9 so that the tension on the filaments between the guide roller 10 and the nip rollers is 0.1 g/denier or above.

It is preferred that one or more of the heating rollers 3 to 9 should be used for cooling purposes. The number of the cooling rollers is properly chosen. Hot plates or hot vapor may also be used as the heating or cooling medium. The use of rollers is advantageous in that a larger length of contact between the roller and the filaments can be obtained with the need for a smaller space.

The following Examples will illustrate the present invention.

## EXAMPLE 1

A 500,000 denier undrawn polyethylene terephthalate tow was drawn at a draw ratio of 3.80 at 70°C. in a first stage, and then at a draw ratio of 1.20 at 100°C. in a second stage. The tow was then passed over heating rollers of the type shown in the accompanying drawing, and then fed into a stuffer crimper where it was crimped. The heating rollers 3 to 7 were used for heat-treating purposes, and the heating rollers 8 and 9, for cooling purposes. The experiments were performed at varying roller temperatures. The tension of the tow was 1.5 g/denier between the roller 3 and the cooling roller 9, and 1.0 g/denier between the guide roller 10 and the nip rollers 11 and 11'. The results are shown in Table 1.

The percentage crimp, the number of crimps, and Young's modulus were measured by the following methods.

## PERCENTAGE CRIMP

The specimen filament of a given length (a) is placed under an initial load of 2 mg/denier. Then, a load of 50 mg/denier is exerted on the filament, and the length (b) of the filament is measured after the lapse of 30 seconds. The percentage crimp is expressed by:

$$(b - a)/b \times 100 \text{ (percent).}$$

## NUMBER OF CRIMPS

The number of buckling points over a length of 25 mm under a load of 2 mg/denier is counted, and this value is divided by 2. The value obtained gives the number of crimps per 25 mm since the number of buckling points is twice as great as that of crimps.

## YOUNG'S MODULUS

The stress-strain curve of the specimen filament is recorded by an Instron tensile tester, and the Young's modulus is calculated from the inclination of the tangent line which provides the maximum gradient on the curve.

The temperature of the filaments at the inlet of the crimper as shown in Table 1 was obtained by measuring the temperature of the filaments immediately before entry to the nip rollers of the crimper using a surface temperature measuring instrument type HP-4F produced by Anritsu Meter Mfg., Co.

It is clear from the results given in Table 1 that polyester filaments having sufficiently high Young's modulus cannot be obtained at temperatures below 135°C., and when the heat-treatment temperature is 250°C., the undesirable melt-adhesion of the individual filaments occurs. The results of the comparison 2, 3 and 4 show that unless the temperature of the filaments immediately before entry into the crimper is kept at least 10°C. lower than the heat-treating temperature and between 100°C. and 140°C., both the crimpability and Young's modulus cannot be improved at the same time.

## EXAMPLE 2

Crimped polyester filaments were produced under the same conditions as used in the preparation of the filaments in Run 5 of Example 1 except that the tension of the yarn was the same both at the time of the heat-treatment under tension and at the time of cooling treatment, and this tension was varied as shown in Table 2 below. The properties of the filaments obtained are shown in Table 2 below.

Table 2

| Run Nos.   | Tension of the yarn (g/den) | Number of crimps per crimp 25 mm (%) | Young's modulus (kg/mm <sup>2</sup> ) |
|------------|-----------------------------|--------------------------------------|---------------------------------------|
| 5-1        | 1.0                         | 13.1 15.6                            | 730                                   |
| 5-2        | 0.6                         | 12.6 14.2                            | 680                                   |
| 5-3        | 0.4                         | 13.0 13.3                            | 600                                   |
| Comparison | 0.25                        | 12.8 11.6                            | 510                                   |

It is seen from the results shown in Table 2 that the tension of the yarn at the time of the heat-treatment must be at least 0.3 g/denier, preferably at least 0.5 g/denier, and when the tension is reduced to 0.25 g/denier, the Young's modulus decreases, and filaments having high Young's modulus cannot be obtained.

## EXAMPLE 3

Crimped polyester filaments were produced under the same conditions as shown in Runs Nos. 1 and 7 in Example 1 except that the tension of the yarn between the heating roll 9 and the nip rollers of the crimper was changed as follows: (a) reduced to 0.5 g/denier, (b) reduced to 0.2 g/denier, (c) reduced to 0.1 g/denier, (d) reduced to 0.05 g/denier, and (e) reduced to 0.05 g/denier and then elevated to 0.5 g/denier. The percentage crimp and the number of crimps of each of the filaments obtained were measured and shown in Table 3.

TABLE 1

| Run numbers       | Temperature of heating rollers 3 to 7 (°C.) | Temperature of heating rollers 8 and 9 (°C.) | Temperature of the tow at the inlet of crimper | Number of crimps per 2.5 cm.  | Percentage crimp (percent) | Young's modulus (kg./mm. <sup>2</sup> ) |  |
|-------------------|---------------------------------------------|----------------------------------------------|------------------------------------------------|-------------------------------|----------------------------|-----------------------------------------|--|
| Comparison 1..... | 125                                         | 115                                          | 111                                            | 13.0                          | 13.0                       | 580                                     |  |
| 1.....            | 135                                         | 115                                          | 110                                            | 12.8                          | 14.3                       | 710                                     |  |
| 2.....            | 135                                         | 125                                          | 119                                            | 13.1                          | 12.3                       | 660                                     |  |
| Comparison 2..... | 135                                         | 135                                          | 129                                            | 12.9                          | 12.1                       | 530                                     |  |
| Comparison 3..... | 180                                         | 90                                           | 87                                             | 13.2                          | 10.3                       | 720                                     |  |
| 3.....            | 180                                         | 105                                          | 102                                            | 13.1                          | 12.9                       | 750                                     |  |
| 4.....            | 180                                         | 110                                          | 104                                            | 12.9                          | 13.9                       | 750                                     |  |
| 5.....            | 150                                         | 120                                          | 113                                            | 13.3                          | 15.8                       | 780                                     |  |
| 6.....            | 170                                         | 130                                          | 121                                            | 13.0                          | 15.4                       | 860                                     |  |
| 7.....            | 170                                         | 140                                          | 136                                            | 13.1                          | 14.0                       | 850                                     |  |
| Comparison 4..... | 170                                         | 155                                          | 147                                            | 13.0                          | 12.4                       | 570                                     |  |
| 8.....            | 230                                         | 130                                          | 120                                            | 12.8                          | 12.4                       | 830                                     |  |
| Comparison 5..... | 250                                         | 130                                          | 118                                            | Melt adhesion occurred partly |                            |                                         |  |

TABLE 3

| Properties | Run No. 1                    |                            |                                         | Run No. 2                    |                             |                                         |
|------------|------------------------------|----------------------------|-----------------------------------------|------------------------------|-----------------------------|-----------------------------------------|
|            | Heat-treating temperature    |                            |                                         |                              |                             |                                         |
|            | 135° C.                      | 170° C.                    |                                         | 115° C.                      | 140° C.                     |                                         |
|            | Number of crimps per 2.5 cm. | Percentage crimp (percent) | Young's modulus (kg./mm. <sup>2</sup> ) | Number of crimps per 2.5 cm. | Percentage crimps (percent) | Young's modulus (kg./mm. <sup>2</sup> ) |
| (a)-----   | 12.8                         | 13.8                       | 680                                     | 13.1                         | 13.6                        | 770                                     |
| (b)-----   | 13.1                         | 13.4                       | 670                                     | 13.2                         | 12.0                        | 710                                     |
| (c)-----   | 13.0                         | 12.3                       | 620                                     | 13.0                         | 11.3                        | 640                                     |
| (d)-----   | 12.9                         | 11.1                       | 560                                     | 13.0                         | 9.7                         | 580                                     |
| (e)-----   | 13.0                         | 11.3                       | 520                                     | 12.8                         | 9.6                         | 560                                     |

The results shown, in Table 3 demonstrate that when the tension of the yarn is once reduced as in (d) and (e), the relaxation of the strain of the filaments rapidly proceeds, and it becomes difficult to impart good crimps to the filaments and at the same time, the Young's modulus is reduced.

What we claim is:

1. A process for producing polyester filaments having high Young's modulus and excellent crimps, which comprises heat-treating a bundle of drawn filaments of a substantially linear, fiber-forming, high-molecular-weight polyester in which at least 85 mole percent of the recurring units consist of ethylene terephthalate, at a temperature of 135° to 240°C. under a tension of at least 0.3 g/denier; feeding the filaments to the nip rollers of a stuffer box while maintaining the filaments at a temperature at least 10°C. lower than the heat-treating temperature and between 100° and 140°C. under a tension of at least 0.1 g/denier; crimping the filaments in the stuffer box; and then withdrawing the filaments from the stuffer box.

15 2. A process of claim 1, wherein the upper limit of the tension during the heat-treatment is 3.5 g/denier.

3. A process of claim 1, wherein the lower limit of the tension during the heat-treatment is 0.5 g/denier.

4. A process of claim 1, wherein the treating temperature in the heat-treatment step is 150° to 230°C.

25 5. A process of claim 1, wherein the filaments heat-treated under tension are fed to the nip rollers with the temperature of the filaments maintained at at least 20°C. lower than the heat-treating temperature.

25 6. A process of claim 1, wherein the lower limit of the temperature of the filaments fed to the nip rollers is 110°C.

30 7. A process of claim 1, wherein the upper limit of the tension of the filaments fed to the nip rollers is 1.0 g/deier.

30 8. A process of claim 1, wherein the lower limit of the tension of the filaments fed to the nip rollers is 0.2 g/denier.